

# UNITED STATES PATENT OFFICE.

JAMES M. SKINNER, OF PHILADELPHIA, PENNSYLVANIA, ASSIGNOR TO PHILADELPHIA STORAGE BATTERY COMPANY, OF PHILADELPHIA, PENNSYLVANIA, A CORPORATION OF PENNSYLVANIA.

## PROCESS OF TREATING WOOD FOR STORAGE-BATTERY SEPARATORS.

1,098,357.

Specification of Letters Patent.

Patented May 26, 1914.

No Drawing.

Application filed December 26, 1912. Serial No. 738,592.

*To all whom it may concern:*

Be it known that I, JAMES M. SKINNER, of Philadelphia, in the State of Pennsylvania, have invented a certain new and useful Improvement in Processes of Treating 5 Wood for Storage-Battery Separators, whereof the following is a specification.

It is the object of my invention to provide wooden diaphragms to be used as separators between the positive and negative plates of a secondary or storage battery, deprived of the natural constituents of the wood which, if allowed to remain, tend to decompose when immersed in the usual 10 electrolyte, viz., an aqueous solution of sulfuric acid, and subjected to the action of the battery, and form acetic acid or other products which are deleterious to the battery. Such deleterious constituents of the 15 natural wood are principally contained in its lignone; the formation of acetic acid and other acids of like nature being a characteristic of such decomposition of lignone. For instance, acetic acid may be formed from 20 the wood by simple hydrolysis of lignocellulose, and oxidation of wood nuclei of ketonic or aldehydic structure.

It is characteristic of my invention that the wood is deprived of said deleterious 25 constituents by salts, and that the wood treated therewith may be allowed to dry in the interim between its treatment and its inclusion in a battery, without materially shrinking, warping, or cracking.

Moreover, my invention is advantageous 30 in that separators treated in accordance therewith have greater strength and durability than wood separators treated with the ordinary acid or alkaline processes.

The wood to be treated is cut in suitable 35 forms, approximately plane sheets, and immersed in an aqueous solution of a salt of hydrogen sulfid; for example, sodium sulfid or potassium sulfid. For instance, I have 40 used aqueous solutions of sodium sulfid containing from 2 to 20 per cent. of said salt, and at temperatures from 15 to 100 degrees centigrade. However, I do not wish to limit myself to said percentages or temperatures.

The sulfid solution acts by reason of its 45 mild hydrolyzing effect upon the wood, by combination of the metal of the sulfid with the wood acids, such as acetic acid and other

acids of that series, which are harmful to lead battery plates, and also by reason of 55 its reducing effect. The reducing effects of the sulfid tend to insure complete treatment of the wood by preventing reversal of the process and oxidation of the products.

My improved process is particularly advantageous, as distinguished from other processes of the prior art, in that it produces a strong, durable separator in a very short time. For instance, using a 15 per cent. solution of sodium sulfid at 100 degrees centigrade, a complete treatment may be effected in one hour; the product thereof being mechanically strong and affording long life in a storage battery. In this connection it may be observed that the acid and alkaline processes 65 of the prior art require twenty-four hours or more treatment of the wood unless solutions are employed of such strength that the product is mechanically weakened. The more rapid action of my present process not 70 only produces properly treated separators at less cost than heretofore but requires correspondingly less floor space and treating apparatus.

It may be observed that the sulfid solution 80 is selective in its action in that it extracts from the wood the constituents thereof harmful to a battery, without detrimental attack upon the wood structure.

The wood separators treated as above contemplated may be washed, to free them of 85 said products which are soluble in water, and then dried with or without artificial heat, and with or without pressure. Good results are obtained by laying the separators 90 horizontally in piles, with a weight on top of each pile.

I do not desire to limit myself to the particular salts named or to the precise proportions thereof above stated, or to the particular temperatures named, as various modifications may be made therein without departing from the essential features of my invention as defined in the appended claims.

I claim:—

1. The process of treating wood separators for storage batteries which consists in immersing them in an aqueous solution of sodium sulfid while maintaining said solution at a temperature of from 15 to 100 degrees centigrade; washing from the treated 100 105

wood the products of decomposition effected by the action of said solution; and, drying the wood, under pressure.

2. The process of treating wood separators for storage batteries which consists in immersing them in an aqueous solution of a salt of hydrogen sulfid while maintaining said solution at a temperature of from 15 to 100 degrees centigrade; washing from the 10 treated wood the products of decomposition effected by the action of said solution; and, drying the wood, under pressure.

3. The process of treating wood separators for storage batteries which consists in 15 immersing them in an aqueous solution of a salt of hydrogen sulfid; washing from the treated wood the products of decomposition effected by the action of said solution; and, drying the wood, under pressure.

20 4. The process of treating wood separators for storage batteries which consists in immersing them in an aqueous solution of a salt of hydrogen sulfid; removing them before the fibers and cells composing them are 25 disintegrated and washing from the treated wood the products of decomposition effected by the action of said solution; whereby said separators are deprived of a portion of their natural constituents harmful to a battery, 30 and are rendered more porous than natural wood, without detrimental attack upon their natural structure.

5. The process of treating wood separators for storage batteries which consists in 35 immersing them in an aqueous solution of sodium sulfid while maintaining said solution at a temperature of from 15 to 100 degrees centigrade; and washing from the treated wood the products of decomposition 40 effected by the action of said solution.

6. The process of treating wood separators for storage batteries which consists in immersing them in an aqueous solution of a salt of hydrogen sulfid while maintaining 45 said solution at a temperature of from 15 to 100 degrees centigrade; and washing from the treated wood the products of decomposition effected by the action of said solution.

7. The process of treating wood separators for storage batteries which consists in 50

immersing them in an aqueous solution of sodium sulfid while maintaining said solution at a temperature of from 15 to 100 degrees centigrade; washing from the treated wood the products of decomposition effected 55 by the action of said solution; and, drying the wood.

8. The process of treating wood separators for storage batteries which consists in immersing them in an aqueous solution of a 60 salt of hydrogen sulfid while maintaining said solution at a temperature of from 15 to 100 degrees centigrade; washing from the treated wood the products of decomposition effected by the action of said solution; and, 65 drying the wood.

9. The process of treating wood separators for storage batteries which consists in immersing them in an aqueous solution of a salt of hydrogen sulfid; washing from the 70 treated wood the products of decomposition effected by the action of said solution; and, drying the wood.

10. The process of treating sheets of wood to deprive them of lignone, without destroying 75 the natural structure of said sheets; which consists in subjecting them to the action of a salt of hydrogen sulfid and then washing them.

11. The process of treating wood separators for storage batteries which consists in subjecting them to the action of a salt of hydrogen sulfid; and eliminating from the 80 wood the products of the resultant reaction, without destroying the natural structure of 85 the wood.

12. The process of treating wood separators for storage batteries which consists in subjecting them to the action of sodium sulfid; and eliminating from the wood the 90 products of the resultant reaction, without disintegrating the fibers of the wood.

In testimony whereof, I have hereunto signed my name at Philadelphia, Pennsylvania, this twenty-first day of December, 95 1912.

JAMES M. SKINNER.

Witnesses:

JOHN S. THOMAS,  
EDWARD S. PEYTON.